

## UNITED STATES PATENT OFFICE.

JOHN HARRIS, OF CLEVELAND, OHIO.

## GASEOUS FUEL.

No Drawing.

Application filed December 6, 1923. Serial No. 678,807.

## To all whom it may concern:

Be it known that I, JOHN HARRIS, a citizen of the United States, residing at Cleveland, in the county of Cuyahoga and State of Ohio, have invented a certain new and useful Improvement in Gaseous Fuel, of which the following is a full, clear, and exact description.

This invention relates to gaseous fuels, 10 and more particularly to a gaseous fuel which, when used in combination with oxygen, is especially adapted for the purpose of cutting metals.

It is the general object of the invention 15 to produce a gaseous fuel which is relatively inexpensive, which will enable the cutting operation to be performed in a most efficient manner, and with the use of a gas which is ordinarily readily obtainable.

20 I prepare a gaseous fuel by which the foregoing general object may be realized by saturating or impregnating natural gas with ordinary commercial ether. The most convenient manner in which this saturation or 25 impregnation may be accomplished is by introducing into a cylinder containing about 200 cu. ft. of natural gas, about one to two pounds of commercial ether. When the delivery valve from such a tank is opened, the 30 natural gas, impregnated with the ether, will be supplied to the blowpipe and the latter may be operated with oxygen in the usual manner.

When the ether is added to and mixed 35 with the natural gas in the manner set forth hereinbefore, the resultant gaseous fuel will consist of approximately 97½ to 95 parts by volume of natural gas, to approximately 2½ to 5 parts by volume of ether vapor.

40 The advantage of my fuel mixture is that the ether increases the flame temperature and the heat units of the natural gas. Furthermore, by reason of the fact that it lowers the igniting point of the natural gas, 45 the mixture can be used with ordinary blowpipe tips, without danger of the flame being blown off such tips, as is the case where natural gas is attempted to be used without dilution with such heavier hydrocarbon—

tips intended for burning natural gas have 50 to be provided with special cups for the prevention of this blowing out or blowing off of the preheating flame.

By the use of my invention, the natural gas can now be used with the same facility 55 as ordinary cutting gases, but at much less cost and with greater efficiency.

Where one pound of ether is employed with a cylinder of gas, the resultant gas will realize all of the advantages set forth hereinbefore; where two pounds of ether are employed with a cylinder of gas, a corresponding increase in flame temperature and heat units will be realized, with a corresponding 60 increase in the speed of cutting, and the igniting point will be further lowered, thus insuring the maintenance of the flame at the blowpipe tips without liability of being blown off. Furthermore, with the higher 65 limit or larger quantity of ether, the gas is particularly useful for cutting heavy masses 70 of metal or dirty metal with great facility.

While commercial or ethyl ether is preferred for admixture with natural gas, because of its richness in carbon and hydrogen. 75 my invention contemplates the use of methyl ether, as well, for such admixture.

Having thus described my invention, what I claim is:—

1. A gaseous fuel particularly useful for 80 the cutting of metal and consisting essentially of a mixture of natural gas with the vapor of ether in the proportions of not materially less than 2½ to not materially greater than 5 parts by volume of the ether vapor, 85 to from not materially greater than 97½ to not materially less than 95 parts by volume of said natural gas.

2. A cutting gas consisting essentially of 90 natural gas having mixed therewith vapor of ether, said vapor constituting not materially less than 2½% by volume of the mixture and the natural gas constituting not materially more than 97½% by volume of the mixture.

In testimony whereof, I hereunto affix my signature.

JOHN HARRIS.